

## UNITED STATES PATENT OFFICE.

LINWOOD M. BROWN, OF PITTSBURGH, PENNSYLVANIA.

## STEEL ALLOY.

No Drawing.

Application filed February 14, 1927. Serial No. 168,828.

My invention relates to steel alloys, and more particularly to the class of steel alloys used in making cutting tools.

One object of the invention is to provide a steel alloy which combines increased strength and toughness with improved hardening, cutting and percussive qualities.

Another object of the invention is the provision of a steel alloy which readily permits of the heat treatment to which such alloy steels are subjected throughout a wide range in temperatures.

With this and other objects in view, the invention consists in a steel alloy of the composition and ranges in proportions hereinafter described and particularly specified in the appended claims.

In making my improved alloy, which preferably will be made in an electric furnace, the alloying elements and approximate ranges in proportions by weight of the various elements in the finished alloy will be substantially as follows—

|                                     | Per cent.    |
|-------------------------------------|--------------|
| 25 Carbon                           | 0.40 to 1.00 |
| Manganese                           | 0.50 to 1.50 |
| Silicon                             | 1.50 to 2.50 |
| Molybdenum                          | 0.15 to 1.50 |
| Vanadium                            | 0.15 to .50  |
| 30 Combined molybdenum and vanadium | .50 to 1.00  |

The impurities, phosphorous and sulfur, will be .04 per cent or under, and the iron content will be sufficient to make 100 per cent.

In addition to the above alloying elements uranium, in amounts of from .15 to .50 per cent may be added, the amount of iron in the composition being correspondingly lessened. When used, the uranium will replace a corresponding amount of molybdenum or vanadium or part of each of these two elements.

45 The carbon, manganese and silicon will be added to the bath in the furnace, and the

molybdenum and vanadium additions preferably, although not necessarily, will be made in the ladle. When used the uranium will be added to the metal in the ladle. 50

In making my improved steel alloy, ferro-alloys of silicon, manganese, molybdenum, vanadium and uranium will be found best for use.

The advantages of my invention result 55 from the use in a high silicon alloy of the molybdenum and vanadium with the other alloying elements within the range in proportions specified. Alloys made in accordance with my invention have very great 60 resistance to crystallization or fatigue and are particularly well adapted for use as rock drills and similar percussive tools.

Many variations in the proportions of the alloying elements may be made without departing from my invention as defined in the appended claims.

I claim—

1. A steel alloy containing from 0.40 to 1.00 per cent carbon, from 0.50 to 1.50 per 70 cent manganese, and having from 1.50 to 2.50 per cent silicon, 0.70 per cent molybdenum and 0.70 per cent vanadium alloyed therewith.

2. A steel alloy containing from 0.40 to 75 1.00 per cent carbon, from 0.50 to 1.50 per cent manganese, from 1.50 to 2.50 per cent silicon, and a combined molybdenum and vanadium content of from 0.50 to 1.00 per cent and having at least .15 per cent molybdenum or vanadium. 80

3. A steel alloy containing from .40 to 1.00 per cent carbon, from .50 to 1.50 per cent manganese, from 1.50 to 2.50 per cent silicon, a combined molybdenum and vanadium content of from .50 to .70 per cent and having at least .15 per cent of molybdenum or vanadium. 85

In testimony whereof I have hereunto signed my name.

LINWOOD M. BROWN.